

[54] **METHOD OF MAKING METAL FOAMS BY  
SEQUENTIAL EXPANSION**[75] Inventors: **Leonard M. Niebylski, Birmingham;**  
**Chester P. Jarema, Detroit, both of**  
**Mich.**[73] Assignee: **Ethyl Corporation, Richmond, Va.**[22] Filed: **June 21, 1971**[21] Appl. No.: **155,210****Related U.S. Application Data**[63] Continuation-in-part of Ser. No. 879,515, Nov. 24,  
1969, abandoned.[52] **U.S. Cl. .... 75/20 F, 75/20 R, 75/86**[51] **Int. Cl. .... C21b**[58] **Field of Search .... 75/20 F, 20 R, 86**[56] **References Cited****UNITED STATES PATENTS**

|           |         |                    |           |
|-----------|---------|--------------------|-----------|
| 2,937,938 | 5/1960  | Fiedler et al..... | 75/20 R   |
| 3,214,265 | 10/1965 | Fiedler .....      | 75/20 R   |
| 3,300,296 | 1/1967  | Hardy et al. ....  | 75/20 R   |
| 3,305,902 | 2/1967  | Bjorksten .....    | 75/20 R X |

*Primary Examiner—L. Dewayne Rutledge**Assistant Examiner—W. R. Satterfield**Attorney, Agent, or Firm—Donald L. Johnson; Robert  
A. Linn*[57] **ABSTRACT**

Metal foams are produced by decomposing a blowing agent in a molten metal such that there is an initial and a subsequent expansion due to blowing gas. The sequential expansion can be conducted by more than one addition of blowing agent to the molten metal to be expanded, or by allowing the molten mass to expand, applying agitation to collapse the foam, and allowing it to expand again, or by forming an intermediate product by expanding and cooling, remelting the intermediate, stirring, and foaming again. Zinc-based foams of fine quality are produced. In a preferred embodiment, substantially pure zinc, titanium hydride (0.1 to 1.5 weight per cent based on weight of metal, and a reaction temperature of from about 475° to about 500°C. are employed.

**4 Claims, No Drawings**

## METHOD OF MAKING METAL FOAMS BY SEQUENTIAL EXPANSION

This is a continuation-in-part of application Ser. No. 879,515, filed Nov. 24, 1969 now abandoned.

### BACKGROUND OF THE INVENTION

Foamed metals have been described in the prior art; see for example, U.S. Pat. Nos. 2,895,819, 3,300,296, and 3,297,431. Such foams are produced by adding a gas-evolving compound to a molten metal and thermally decomposing the compound to evolve blowing gas. The gas forming compound can be a metal hydride such as  $ZrH_2$  or  $TiH_2$ ; U.S. Pat. No. 2,983,597.

It is known that zinc foams can be produced; confer the aforementioned U.S. patents. In those patents, alloys having an appreciable amount of metal other than zinc are taught to form foams. This invention provides means to foam substantially pure zinc as well as other metals and alloys.

### SUMMARY OF THE INVENTION

In essence, this invention provides metal foams and processes for their formation. In an important aspect, this invention provides a process for preparation of a metal foam, said process comprising decomposing a blowing agent in a molten metal to produce blowing gas such that there is an initial and a subsequent evolution of blowing gas from said blowing agent; and subsequently cooling the expanded mass produced after the final evolution of blowing gas, thereby forming a set cellular product.

Methods for the sequential expansion include more than one addition of blowing agent to the molten metal to be foamed,

allowing the molten mass to expand by decomposition of blowing gas, causing the foam to collapse and expand again, and

forming a set intermediate product by expanding and cooling, remelting the intermediate, and foaming again.

By such techniques, zinc-based metals including substantially pure zinc or alloys having 85 per cent zinc or more, can be efficaciously expanded.

### DESCRIPTION OF PREFERRED EMBODIMENTS

In a preferred embodiment, substantially pure zinc is employed as the metal to be foamed. Zinc alloys having up to about 15 weight per cent of alloying metal(s) such as aluminum-zinc and magnesium-zinc alloys can be used. Typical alloys which can be employed are ZDC No. 3 (AG40A), ZDC No. 5 (AC41A) and Alloy ZDC No. 7. Compositions of such alloys are set forth on pages 28-9 of *ASARCO, Zinc Die Casting Alloys*, American Smelting and Refining Company Bulletin VII-I. The compositions of those alloys recited on the cited pages are incorporated by reference herein as if fully set forth. Another typical alloy is ILZRO 12; it has the composition

aluminum — 11-13 percent  
copper — 0.5-1.25 percent  
magnesium — 0.01-0.03 percent  
zinc — balance

Also lead-zinc alloys can be foamed according to the process of this invention, so long as they are molten at applicable temperatures, such as the ranges discussed below. Moreover, this invention can be extended to

lead and lead alloys. The lead may be alloyed with magnesium or aluminum. Other alloys can be employed as well as other substantially pure metals.

The temperature employed is not a truly independent variable but is dependent at least in part on the nature of the metal and the nature of the blowing agent employed. The temperature employed is an elevated temperature sufficient to maintain the metal in a molten state while expansion takes place and also sufficient to thermally decompose the blowing agent to form blowing gas at a rate which yields foaming at the desired speed. The speed of foaming should not be so long as to unduly delay the process; likewise, it should not be too fast for blow-hole formation or other untoward event may occur. Usually it is desirable to employ a temperature which allows the sum of the plurality of expansion periods to total from about 1 to about 45 minutes, but shorter and faster times can be employed. Given a desired metal-blown agent system, a skilled practitioner can determine a desired temperature and suitable expansion time sum with a minimum of experimentation. Preferred sums are 2-30 minutes and most preferred from about 3 to about 15 minutes. Thus, temperatures of 395°-655°C. can be employed and it is preferred to use temperatures of from about 425° to about 625°C. More preferable, temperatures of from about 425° to about 525°C. and most preferably from about 475° to about 500°C., are employed.

Such temperatures are conveniently used when conducting the process by utilizing a metal hydride such as magnesium or titanium hydride as the blowing agent. In general, for this invention, hydride blowing agents are of choice. The titanium hydride of commerce usually has a little less hydrogen than the stoichiometric amount. Such commercial material is very satisfactory, as are materials wherein more hydrogen has been removed (by treatment at about 400°C. for from about 1 to 24 hours). When foaming a zinc-based metal, that is, a metal which has 85 weight per cent zinc or more, titanium hydride affords a finer pore structure than  $MgH_2$ .  $ZrH_2$  prepares foams usually of intermediate pore size. Thus, where coarser zinc-based foams are desired,  $MgH_2$  is preferred over titanium hydride. As with the process temperature, preferable blowing agents for other metals can be found with minimum testing.

The amount of blowing agent is, in general, dependent upon the amount of expansion desired. To achieve foams of equivalent densities from different metals may require different amounts of blowing agents. For example, about 7 weight per cent of  $TiH_2$  will give a very light zinc foam and a much heavier lead foam.

In general, from about 0.1 to 1.5 weight per cent of blowing agent is utilized in the process of this invention. However, greater and lesser amounts can be employed if desired. As the amount of blowing agent increases (when other parameters are allowed to remain constant) preparation of less dense foams is favored. When using titanium hydride, a preferred amount is from about 3 to about 10 grams per each 1,000 gram portion of zinc-based metal to be foamed.

As taught above, the process of this invention entails more than one expansion of a molten mass utilized to form a set cellular product. In a preferred embodiment, two expansions are employed, that is, an initial expansion is followed by a final expansion. If desired, more than two expansions can be carried out. Thus, three, four or more expansions may be used.

When the process is conducted, all the blowing agent to be employed can be introduced by one addition. When this expedient is employed, one method of achieving a plurality of expansions is to allow the material to foam, then cause the foam to collapse, and then allow the molten mass (thereby produced) to foam again. Good results are obtained when the initial expansion increases the mass to be foamed from about two to about three times the original volume, and the foam is made to collapse to the original volume or thereabouts, say, up to about 1.1 or 1.2 times the original volume.

The foam can be made to collapse by stirring as described above, however, it is not necessary to do so.

One can add all the blowing agent in one addition, allow the molten mass to foam, cool to form an intermediate set cellular product, remelt and stir, and allow the mass to foam again, and then cool to form a final set cellular product. This embodiment can be carried out in a number of ways. For example, a comparatively large amount of blowing agent can be added, say up to about 5 to about 10 weight per cent based on weight of metal to be formed, allow the molten mass thus formed to foam to an extent greater than desired for the final product, cool to form an intermediate, and then remelt and stir, and finally, allow the molten mass to foam to the extent desired. Alternatively, after the original addition of blowing agent, the foaming can be stopped with less or about the same amount of foaming as desired in the final product. These products can be remelted and refoamed as pointed out above. Moreover, one can make one addition of blowing agent, allow the first expansion to take place to the extent desired, cool and add some or all the intermediate thereby produced to a further amount of molten metal, allow foaming to occur to the desired extent, and then allow the final product to cool and set. Routine experimentation can determine the extent of initial expansion and the amount of non-blown molten metal which will yield a desired product for any given amount of blowing agent and initial amount of molten metal used to form the intermediate product.

Alternatively, the blowing agent employed may not all be added in one addition. In other words, a plurality of additions of blowing agent can be utilized. Good results are achieved using two blowing agent additions, but more can be employed if desired. Thus, one can make three, four or five or even more separate additions of blowing agent to the molten mass. When using two additions, generally at least 5 weight per cent of the total amount of blowing agent to be employed is added in the first addition. In some instances, it is desirable to add at least 10 percent of the blowing agent. In many instances it is desirable to add about 50 per cent of the blowing agent in the first addition. Greater or lesser amounts than those discussed above can be added in the first addition, as desired.

The blowing agent need not be added to the molten metal at the same temperature. In fact, in a preferred embodiment of this invention using zinc-based foams, a portion of the blowing agent is added at a temperature of from about 425° to about 450°C. and subsequently the remainder of the blowing agent is added at a temperature of from about 475° to about 525°C. When this operation sequence is employed, foaming occurs over a longer period of time and more uniform mixing of the blowing agent in the molten metal can be

achieved. These beneficial results are enhanced by the temperatures of 425° – 450°C., since that usually affords very slow foaming.

The above embodiments may be combined. For example, one can add blowing agent to a molten mass, allow it to foam to form an intermediate set cellular product, remelt, add a second quantity of blowing agent, allow the mass to foam to the desired extent, and then cool to form the final set cellular product.

For the process of this invention to achieve its best results, it is desirable that the initial expansion occur to a significant amount. The exact amount of initial expansion required per given embodiment and per given amount of blowing agent in molten metal can be determined for each agent and metal via routine experimentation. Generally, good results are achieved if upon initial expansion the molten mass expands to form about two to three times the initial volume. Greater or lesser amounts of expansion can be employed. For example, good results can be achieved when the initial expansion occurs to about 110 per cent of the initial volume. Similarly, good results have been achieved when the initial expansion was about 15 times the original volume and three times the final volume. Thus, the final expansion can be to a greater or lesser extent than a previous expansion. When an intermediate set cellular product is to be formed and this is to be added to additional molten metal (and no more blowing agent is to be added to the final melt) the amount of initial expansion, generally, is equivalent to about 1.1 to about three times the volume of the final amount of molten metal.

The ability to form satisfactory foams utilizing an initial expansion followed by a cooling step to form an intermediate set cellular product has two advantages. First, it allows scrap foam to be utilized. Second, it allows the formation of set cellular product at one location and shipment to another for final expansion.

In an important aspect, this invention involves the discovery that better results are achieved if the molten mass to be foamed had been subjected to an initial prior treatment with blowing gas. The reason for the beneficial result obtained is not known with certitude. Not wishing to be bound by any theory, the beneficial result may occur through increased wetting of the blowing agent employed. It has been noted that in certain metals such as zinc, upon initial addition of blowing agent such as titanium hydride, that even after rapid, efficient stirring, some metal hydride particles will come to the surface of the molten metal. If the molten metal is subjected to an initial addition of titanium hydride followed by sufficient stirring and some expansion as described above, it has been noted that there is generally much less blowing agent on the surface after a second addition of blowing agent. These results tend to hypothesize that pre-gassed metal may have an enhanced ability to wet blowing agent particles such as metal hydrides.

In a preferred embodiment, the temperature of the mass to be foamed with  $TiH_2$  is maintained by an induction field. For reasons unknown to us, it appears that induction heating affords higher quality foams than resistance heating methods. In addition, induction heating affords closer process control.

As appreciated by a skilled practitioner, better foams are produced if the blowing agent is substantially uniformly mixed throughout the molten metal to be foamed. Thus, we prefer to use mixing techniques

which tend to give efficient mixing. High speed stirring is a method of choice.

Our process proceeds well at ambient pressure, but greater and lower pressures can be used if desired.

The following exemplary material serves to illustrate the process of this invention.

#### EXAMPLE I

In a cylindrical reaction vessel, a 1,200 gram charge of substantially pure zinc was heated to 440°C. To this was added four grams of  $TiH_2$  enclosed within lead foil. The addition of titanium hydride was carried out while dispersing, using high speed mixing, for approximately 30 seconds. Very slight foaming occurred. An additional 5 gram portion of titanium hydride was added and stirred in for approximately 30 seconds while the molten metal was at a temperature of 470°C., utilizing an induction field. While this temperature was maintained, foaming continued for 4-5 minutes. Upon cooling, a good quality foam of 12-13 per cent density with very small (1/64-1/32 inch) average pore size cells was produced.

Similar foams are made when the amount of titanium hydride is from 1 to 15 grams per 1,000 gram portion of zinc. Similar foams are also produced when the same amounts of magnesium hydride are employed but in general they have larger pores than analogous  $TiH_2$  foamed materials. Likewise, analogous foams are produced from zinc alloys having up to about 15 weight per cent of alloying material selected from magnesium, aluminum, zinc, and combinations thereof. Similar foams are produced when the process of the above invention is continued at temperatures up to about 625°C. However, the foaming is more rapid and in many instances, greater amounts of blowing agent are preferably employed.

Our work has indicated that zinc foams are made in fine pore qualities only if they have been subjected to at least two foam operations. If only one expansion is allowed to take place, the resultant foam will be large celled, non-uniform, and will usually have a heavy skin bottom. Such inferior foams can be produced for example, using pure zinc and 0.75 - 1.25 grams of titanium hydride per each 100 gram portion of zinc employed.

#### EXAMPLE II

A 1,120 gram portion of substantially pure zinc was melted and 60 grams of substantially pure aluminum were added to the zinc at 450°C. The temperature was raised to 600°C.

Thereafter, the temperature was brought to 460°C. and 10 grams of  $TiH_2$  were mixed with the Al-Zn alloy. The temperature dropped to 420°C., and in spite of admixing with efficient stirring, some of the hydride remained on top of the alloy. The resultant mixture was reheated such that it reached 480°C. In approximately 5 minutes. During this reheating, it foamed slowly.

The foam was restirred such that the melt approached the initial volume and reheated to 480°C. After 4 minutes at this temperature foaming stopped.

The crucible containing the molten mass was removed from the induction furnace. It was noted that some foam collapse had occurred. Sectioning revealed collapsed cells and a 1/2 inch thick bottom skin.

#### EXAMPLE III

A 953 gram portion of substantially pure zinc was melted and 43 grams of substantially pure aluminum were added thereto at 450°C. The temperature of the resultant mass was raised to 600°C. to insure alloying.

The temperature was subsequently brought to 500°C. and solid carbon dioxide snow was added to the molten mass until the temperature decreased to 400°C. At that temperature the metal was too cold to add any more carbon dioxide snow. A total of 119 grams of  $CO_2$  had been added. The resultant melt was heated to 600°C. and an additional 132 grams of  $CO_2$  were added. This brought the temperature to 485°C. and the molten metal was very thick.

At 470°C., 10 grams of titanium hydride were added. The metal appeared cold as many solids had formed. The melt was reheated for 2 minutes and at a temperature of 490°C. Foaming occurred until the volume was about twice the original volume. The mixture was restirred until the volume approached the original; the metal was very 'heavy' and as a result mixing was difficult. The induction field was applied again, foaming reoccurred and when the foam reached about 2 inches from the top of the crucible containing it, the crucible was removed from the induction furnace.

Upon standing the foam shrank somewhat. Sectioning revealed a better foam quality than that obtained in Example II. Cell collapse was minimal and the bottom was one-eighth inch as compared to the 1/2 inch skin in Example II. Thus, carbon dioxide improves the quality of aluminum-zinc foams. Similar improvements in quality are achieved with water, nitrogen, and argon. Air or oxygen can also be used to increase the viscosity of the melt.

#### EXAMPLE IV

A 1,200 gram portion of zinc balls was melted and the temperature raised to 450°C. At that temperature, two lead foil packets of 5 grams titanium hydride each were added with stirring. The stirrer was removed and the resultant mass was heated for 5 minutes. Very little foaming occurred during that period in which the final temperature was 430°C. The molten mass was reheated to 450°C. and foaming began. The mixture was restirred causing the volume to decrease to about the original volume. Thereafter the stirrer was removed and the resultant mass reheated for 5 minutes at about 480°-500°C. During that period a heavy lid had been placed on the crucible containing the foam. During the resultant second foaming operation, the zinc foamed to fill the crucible and push the lid up. After cooling to obtain a set cellular product, sectioning revealed a very fine pore foam with no appreciable skin. Utilizing this technique such that before the final expansion the mixture is allowed to foam to 2-3 times the original volume affords good results.

#### EXAMPLE V

A 998 gram portion of zinc ingot was melted and the temperature raised to 460°C. At that temperature 10 grams of titanium hydride (2 lead foil packets) were stirred into the molten zinc. The melt crucible was removed from the induction field and the resultant mass poured into a mold which had been preheated to 475°C. The resultant mixture was not homogeneous.

After 5 minutes in an oven, it was noted the foam had a purplish color; after 8 minutes, the foam was found to have collapsed somewhat. Sectioning after cooling revealed collapsed cells.

A 960 gram portion of the intermediate foam pro-

5 per cent zinc.

Compressive strengths of various zinc foams produced as taught above were determined as indicated in the following table.

The above data are quite variable and this is probably

Compressive Strengths of Various 1" x 1" x 1" Zinc Foams

| Foam Description                                    | Wt.   | (pcf) | Comp. Strength (psi) | Strength to Weight Ratio in psi/pcf |
|-----------------------------------------------------|-------|-------|----------------------|-------------------------------------|
| Pure Zn w*/TiH <sub>2</sub>                         | 4.2g  | 16.0  | 56                   | 3.50                                |
| Do.                                                 | 4.5g  | 17.1  | 56                   | 3.27                                |
| Do.                                                 | 4.2g  | 16.0  | 55.8                 | 3.49                                |
| Pure Zn w/CO <sub>2</sub> and TiH <sub>2</sub>      | 3.7g  | 14.1  | 43.8                 | 3.12                                |
| Do.                                                 | 5.2g  | 19.8  | 60.0                 | 3.03                                |
| 5% Al-95% Zn w/CO <sub>2</sub> and TiH <sub>2</sub> | 9.9g  | 37.7  | 328                  | 8.70                                |
| Do.                                                 | 10.6g | 40.4  | 433                  | 10.7                                |
| Alloy No. 5 w/TiH <sub>2</sub>                      | 11.0g | 41.9  | 317                  | 7.56                                |
| Do.                                                 | 13.4g | 51.1  | 698                  | 13.7                                |
| 3% Mg-97% Zn w/TiH <sub>2</sub>                     | 15.2g | 57.9  | 345                  | 5.96                                |
| Do.                                                 | 16.9g | 64.4  | 872                  | 13.5                                |
| 3% Mg-97% Zn w/ZrH <sub>2</sub>                     | 21.7g | 82.7  | 2000                 | 24.2                                |

\*w=with

duced above was melted and began to foam around 450°C. Stirring was conducted, the stirrer was removed and the induction field applied to give a temperature of about 480°C. At that temperature foaming occurred again and the induction field was shut down. The resultant mass was air cooled and sectioning revealed a very fine pore uniform foam. Density was 48.3 pcf, 11 per cent metal density.

Although a wide variety of blowing agents can be employed, metal hydrides are a preferred class of blowing agents for use in this invention. Of the metal hydrides, magnesium hydride, zirconium hydride, and titanium hydride are preferred since they decompose with enough rapidity to enable foaming to take place at desirable temperatures. In this regard, magnesium hydride will ordinarily liberate enough gas to foam a metal mass at 375°-400°C. and higher, titanium hydride will do so at 435°-450°C. and higher, and zirconium hydride at 465°-485°C. and higher. In general, best results are obtained in this invention with the above blowing agents by utilizing a molten metal at a temperature within from about 20° to about 70°C. of the lower temperature cited above for the selected blowing agent. More preferably, the molten metal should be generally about 50°C. above the lower temperature. Utilizing this temperature-blowing agent relationship, good results are obtained utilizing magnesium hydride, zirconium hydride or titanium hydride in processes similar to the above examples employed with many diverse metals and alloys. Suitable alloys may be binary, ternary or quaternary. Such combinations of lead, zinc, magnesium, tin, silicon, copper and aluminum are useful in this invention. We can use the low melting eutectic of 32 per cent Al and 68 per cent magnesium.

Ternary systems applicable for this invention include combinations of the above named metals exemplified by aluminum-magnesium and silicon. Thus, we can use an alloy with about 3 to about 15 per cent silicon and 0.4-10 per cent magnesium, the balance being aluminum. Other ternary systems which we can use are Al-Cu-Mg, Al-Zn-Mg and the like. Quaternary mixtures include combinations of the above named metals. Typical alloys of this type are Al-Mg-Cu-Zn such as Al 78.5 per cent, Mg 5 per cent, Cu 5 per cent, and 11.5 weight

25 due to the small sample size. Nevertheless, trends can be ascertained. These results indicated that although zinc alloys of aluminum and magnesium are more difficult to foam than pure zinc, such alloys have a much better strength to weight ratio than substantially pure zinc foams. The results also indicate that carbon dioxide thickening of pure zinc produces a foam having a strength-weight ratio about the same as a non-thickened pure zinc foam. Also, the data indicate that 30 magnesium or aluminum additions to zinc tend to cause foam embrittlement.

35 The foamed products of this invention can be utilized in many instances wherein the non-foamed base metals are employed. Foamed zinc can be utilized in structural materials where zinc is now used and less weight is desirable. The zinc foams of this invention can be used in injection molding and diecasting complex shaped hardware for automobiles, aircraft, and other vehicles. For 40 structural use, slabs of foam can be made by pouring the mixture to be foamed into a mold having a flat surface. If the mold surface has a temperature of, say, 50° to 100°C. below the temperature of the expanded mass, then a skin of non-cellular metal can be formed on the foamed mass. Similar conditions hold for lead and lead alloy products of this invention. The lead and lead alloy foams of this invention lend themselves well to use as 45 acoustical materials.

We claim:

- 50 1. Process for preparing a metal foam, said method comprising
- decomposing a blowing agent in a molten metal thereby producing gas which expands said molten metal to about two up to about three times the initial volume of said molten metal,
  - collapsing the foamed mass to about the initial volume of the molten metal by agitation with stirring means,
  - heating to re-expand said molten metal, and
  - cooling the re-expanded mass to form a set cellular product.
- 55 2. A process of claim 1 wherein said metal is a zinc-based metal having up to about 15 weight percent of one or more alloying metals.
- 60 3. A process of claim 1 wherein substantially pure zinc is employed.
- 65 4. Process of claim 1 wherein said blowing agent is selected from the class consisting of magnesium hydride, zirconium hydride, and titanium hydride.

\* \* \* \* \*

UNITED STATES PATENT OFFICE  
CERTIFICATE OF CORRECTION

Patent No. 3,790,365 Dated February 5, 1974

Inventor(s) Leonard M. Niebylski et al

It is certified that error appears in the above-identified patent and that said Letters Patent are hereby corrected as shown below:

Column 1, line 21, should add the following sentence:

-- This is a continuation-in-part of application Serial No. 879,515, filed November 24, 1969, now abandoned. --

Signed and sealed this 15th day of October 1974.

(SEAL)

Attest:

McCOY M. GIBSON JR.  
Attesting Officer

C. MARSHALL DANN  
Commissioner of Patents